

## UNITED STATES PATENT OFFICE.

TENNEY L. DAVIS, OF SOMERVILLE, MASSACHUSETTS.

## EXPLOSIVE.

No Drawing.

Application filed March 8, 1924. Serial No. 697,948.

(GRANTED UNDER THE ACT OF MARCH 3, 1883; 22 STAT. L. 625.)

*To all whom it may concern:*

Be it known that I, TENNEY L. DAVIS, a citizen of the United States, and a resident of Somerville, county of Middlesex, 5 and State of Massachusetts, have invented an Improvement in Explosives, of which the following is a specification.

The invention described herein may be used by the Government, or any of its officers or employees in prosecution of work 10 for the Government, or by any other person in the United States, without payment to me of any royalty thereon, in accordance with the act of March 3, 1883.

15 The subject of this invention is an explosive.

The main object of the invention is the provision of a high explosive suitable for use in boosters, reinforced detonators, detonating fuses, primer caps and as a high 20 explosive either alone or in mixtures with the various substances commonly used in high explosives.

The invention consists specifically, of a 25 new explosive substance, namely, hexanitrocarbanilide, which may also be properly designated hexanitrodiphenyl-urea, or symmetrical di-picryl-urea.

This substance may be prepared by the 30 nitration of carbanilide in one step or in more than one. Carbanilide, formerly prepared by a dangerous process which made use of phosgene, may now be prepared more readily and more simply by a process which 35 I have recently studied which consists in the heating together of aniline and urea.

I do not wish to claim any particular process for the preparation of this explosive for each step in its preparation involves well known chemical procedures.

Pure hexanitrocarbanilide consists of pale yellow crystals which soften at 204° C. and melt with decomposition at 208° C. to 209° C. It yields picric acid when boiled with dilute sulphuric acid and 45 trinitroaniline when boiled with strong ammonia water. It contains 23.25% nitrogen. It is a powerful and brisant high explosive suitable for use in boosters, reinforced detonators, detonating fuses, primer caps, etc., 50 and it may be used alone or in mixtures with other substances for the various purposes to which a high explosive is adapted, as, for example, trinitrotoluene, tetryl, picric acid, etc.

0.19 gram of mercury fulminate is required for the detonation of 0.4 gram of hexanitrocarbanilide. The sand test, carried out in the standard manner specified by the U. S. Bureau of Mines, gave a figure 36.64, slightly better than was given by trinitrotoluene under the same conditions. The drop test was 13 inches, about the same as tetryl, and the temperature of spontaneous explosion was 345° C. as compared with 260° C. for tetryl by the same method.

I claim:

1. An explosive composition having as one of its elements hexanitrocarbanilide.
2. As an explosive, hexanitrocarbanilide

TENNEY L. DAVIS.